

A. J. P. BERTSCHY,  
METHOD AND MEANS FOR CARBURIZING IRON, STEEL, AND ALLOYS THEREOF,  
APPLICATION FILED JAN. 3, 1920.

1,408,686.

Patented Mar. 7, 1922.



Witness:

*Al. Jamieson.*

*By David O. Barnell.*

Attorney.

# UNITED STATES PATENT OFFICE.

ADOLPH J. P. BERTSCHY, OF OMAHA, NEBRASKA.

## METHOD AND MEANS FOR CARBURIZING IRON, STEEL, AND ALLOYS THEREOF.

1,408,686.

Specification of Letters Patent.

Patented Mar. 7, 1922.

Application filed January 3, 1920. Serial No. 349,147.

*To all whom it may concern:*

Be it known that I, ADOLPH J. P. BERTSCHY, a citizen of the United States, and a resident of Omaha, in the county of Douglas and

5 State of Nebraska, have invented certain new and useful Improvements in Methods and Means for Carburizing Iron, Steel, and Alloys Thereof, of which the following is a specification.

10 My invention relates to case-carburizing of iron, steel and alloys thereof, or to methods and apparatus for increasing the carbon content of such materials by treatment at temperatures below the melting-point there-

15 of. It is the object of my invention to provide simple and commercially practicable methods and apparatus for carburizing materials of the class mentioned, whereby a very rapid and uniform penetration of the

20 added carbon may be attained, and wherein it is unnecessary to provide for movement or agitation of the treated articles during the carburizing operation.

In the accompanying drawing I have 25 illustrated diagrammatically an apparatus suitable for carrying out my carburizing process, the figure being a partial longitudinal section of the apparatus.

Referring first to the illustrated apparatus, there is indicated a furnace 1 which 30 will be understood to be heated by any suitable controllable means, such as gas, whereby to maintain the required temperature within the retort 2 in which are placed the

35 articles A to be carburized. The retort 2 extends horizontally through the furnace, and is closed at the rear and front ends, respectively by members 3 and 4, either or both of which may be removable. Said

40 members 3 and 4 are preferably fitted so that a substantially gas-tight joint is provided around them enabling the maintenance of some pressure within the retort, although the use of pressure is not an essential of my

45 carburizing process, and satisfactory work may be produced in a retort having one end, or a substantial part thereof, open to atmosphere. Somewhat more economical control of the process is attained, however, in the

50 closed retort. The front or door-member 4 of the retort is shown as provided with an opening through which a thermo-couple enclosing tube 5 is extended into the retort, the thermo-couple being connected with a suitably calibrated ammeter 6 for indicating temperatures attained within the retort.

The member 4 is also shown as provided with a vent-tube 7, having at the end thereof a cock or valve 8 by which the escape of gases from the retort may be controlled, and 60 a gage 9 for indicating pressures.

The rear end-member 3 of the retort is fitted with a pipe 10, which is shown as carrying at its inner end a downwardly turned elbow 11. The carburizing materials are 65 fed into the retort through said pipe. The carburizing materials employed are mainly or entirely liquid at normal or ordinary atmospheric temperatures, and provision is made for supplying such materials to the 70 feed-pipe 10 as follows: A portion of the pipe is enclosed by a jacket 12, forming around the pipe a chamber 13 through which heating or cooling media may be circulated, through pipes 14 and 15 connecting with the 75 jacket. The portion of the feed-pipe within the jacket forms a multiple header, being branched therein to connect with a plurality of pipes 16, shown as extending vertically through the jacket. Each of said pipes 16 80 has a control-valve 17, and may also be provided with sight-feeding devices 18, through which the dropping of liquids fed through them may be observed. To each of the pipes 16 there is connected a reservoir 19, only one 85 of which is shown complete in the drawing, but all of which will be understood to be alike. To the upper closed end of the reservoir there is connected a pipe 20 through which the reservoir is filled, said pipe having 90 a valve or cock 21 which may be opened or closed as required. To said upper closed end of the reservoir there is also connected a pipe 22 through which air-pressure may be supplied should it be desired to force-feed 95 the material from the reservoir to the pipe 10. The pipe 22 has a lateral branch 23 connecting with a pressure-gage 24 and a blow-off pet-cock 25.

In the use of the described apparatus to 100 carry out my process, the articles A to be treated are placed within the retort preferably being arranged therein with substantial uniformity and held apart by suitable spacing members B. To secure uniform results, 105 none of the articles should be placed in immediate proximity to the end of the feed-pipe, and all of the articles should be in portions of the retort which experience has shown to be capable of being maintained by 110 the furnace at substantially uniform temperature throughout. In general, better

results are attained when the space within the retort is well filled with the treated articles than when said space is only partly filled; providing, of course, that the articles themselves should be slightly separated from each other, and excluding from consideration the space immediately adjacent to the end of the feed-pipe, as well as any portion or portions of the retort which are found to be heated by the furnace abnormally, or to temperatures differing materially from the remaining major portion thereof.

The temperatures to which the retort is heated during the carburizing operation may be varied according to the results desired, the extreme range being from 1400° F. to 1900° F., with a preference in most instances for temperatures ranging from 1700° F. to 1800° F. The lower limit of temperature appears to be the "critical" temperature of the material, at which the contained carbon enters into solid solution, and to which the steel must be heated in order to effect hardening thereof upon quenching. In general, the higher the temperatures the more rapidly the carburizing effects are produced, and the maximum limits of temperature are those which may be attained with the particular material operated upon, without injury thereto.

The particular characteristic of the apparatus employed for carrying out my process, lies in the provision of means for feeding into the retort, with substantial continuity throughout the carburizing period, of carbonaceous materials which are liquid at normal atmospheric temperatures, said materials being fed directly to the retort so as to either enter the same while in the liquid form or to become vaporized only immediately preceding, and substantially upon, their entry into the retort-chamber.

My process is especially characterized by the substantially continuous feeding to the retort, during the carburizing period, of normally liquid carbonaceous material capable of being decomposed at the temperatures maintained within the retort, and the controlling of the rates of feed and escape, and of the maintained temperatures of the retort, such as to establish therein around the treated articles a zone of substantially uniform reaction in which the changes being undergone by the material are favorable to the release therefrom of carbon in such a form or state as to penetrate and combine with the metal in the articles being treated.

The carbonaceous materials suitable for use in the process appear to be any of the higher homologues of the several hydrocarbon series, such as of the paraffin, olefin, acetylene, terpene, benzene, naphthalene, anthracene, or other series. In actual practice I have employed principally petroleum and

the various refined products thereof, and have obtained satisfactory results from the use of such materials, ranging in composition and density from crude oil through the various refined products to kerosene. Besides the usual factors of time and temperature, which control carburizing in other processes, in my process the character of the case obtained upon the treated articles, and the depth of penetration thereof, are varied according to (a) the kind or density of the oil used, (b) the quantity fed per unit of time and proportional to the transverse sectional area of the retort through which the decomposing vapors pass, and (c) the size of the vent through which the evolved gaseous products escape from the retort. The latter factor, when the vent is restricted, may result, of course, in the building up of slight pressure within the retort. Different liquids, such as oils of different densities, may be placed in the several reservoirs 19, and fed to the pipe 10 either simultaneously or alternatively; or oil of the same kind may be placed in two or more of the reservoirs and fed therefrom alternately, the feed from one being started as the other becomes empty, so as to maintain the continuity of feed to the pipe 10, without interruption due to necessity of refilling the reservoir first used.

When using the lighter and more highly refined oils, a cooling medium such as water may be circulated through the jacket-space 13, to prevent heating of the feed-pipe 10 such as might result in vaporization of the oil prior to its entering the retort-chamber. For heavy oils or greases, the flow thereof may be facilitated by circulating a heating medium through the jacket-space. The feeding of the oil into the retort is preferably commenced when the temperature of the latter reaches the lower limit of the effective range, and is continued substantially throughout the period during which the articles are treated. The decomposition of the higher or complex hydrocarbons under the heat to which the same are subject while passing through the retort, results in the formation therein of soot-like particles and flakes, portions of which pass off through the vent, together with gaseous products, and the remaining portions are deposited in the retort in the form of a loose, spongy mass. In general, larger amounts of the spongy deposit are formed with heavier oils and with higher temperatures, than with lighter or more refined oils and lower temperatures. The presence of the spongy deposit in the retort appears to have an influence upon the carburization of the articles treated, although substantially the same results may be attained with oils which produce a scanty deposit of the spongy material, as with heavier oils which cause a profuse deposit of such material. It should be

understood, however, that it is desirable and perhaps necessary to have in the retort a certain amount of the spongy carbon, as it appears that the desired reactions of the 5 carburizing material occur more effectively in the presence of an appreciable quantity of said spongy material. It has been observed that when a retort is kept heated for a considerable period without feeding of oil 10 to renew the spongy deposit, as when the furnace is kept heated for several hours between runs, the character of the deposit is gradually changed, and becomes harder and denser, finally forming a compact coke-like 15 cake which can only be removed from the retort with some difficulty, by forcibly scraping the same off the walls. It appears further that after the described hardening of the deposit has occurred, no effective car- 20 burizing action is attained in the retort until the spongy deposit begins to be built up by the feeding of fresh oil at a suitable rate. Another viewpoint as to the spongy carbon deposit, is to regard the same as an index 25 for the reaction zone in which the most effective carburizing action is attained. Thus, in a retort of a given length, in which the oil is fed at one end and the gaseous products discharged at the other end, should the 30 rate of feed of the oil be made such that the "cracking" of the heavier hydrocarbons is completed and the ultimate products of the reaction attained, or a state of equilibrium reached for the particular temperature, such 35 that there is no deposit of the spongy carbon near the discharging end of the retort, then it is apt to be found that articles disposed in the retort near the discharge end are not carburized uniformly with articles disposed 40 in the zone of deposit of the spongy material. In a retort having an open discharge end, so that the interior may be directly observed, the character of the reaction may be judged by the appearance of the materials in the 45 different portions of the retort. With a proper rate of feed, air is effectively expelled from the retort by the heavy vapors of the oil, which, of course, become ignited and burn as they escape into air at the mouth 50 of the retort. The formation of the sooty particles and their deposit upon the walls of the retort and upon the articles being treated can be clearly seen, and incandescent 55 particles of carbon may be noted in the flame at the mouth of the retort. Thin streams of blue-white vapor are seen to rise from the spongy carbon deposit, and the evolution thereof may be greatly accelerated by mechanically stirring the deposit. With a sub- 60 stantially closed retort, having merely a vent tube for the escape of the gaseous products, as in the illustrated apparatus, the character of the reaction occurring at any time may be judged by the appearance of the escaping 65 vapors, or by the appearance of the flame produced by ignition thereof. A proper rate of feed of the carburizing material to the retort is indicated in this case by the appearance of a moderate amount of sooty particles at the end of the vent-tube, giving 70 the escaping material a black smoky appearance, and the flame when ignited at the end of the vent-tube has a central reddish luminous cone in which the larger carbon particles form bright points, while the outer 75 portions of the flame are noticeably bluish-white. An excessive feed is indicated by a brown color of the unignited escaping material at the vent, and insufficient feed is indicated by the disappearance or scantiness 80 of the carbon-particles.

The control of the reactions occurring in the retort is closely comparable to that employed in the "cracking" of petroleum and the like, for the production of gasoline, benzene, toluene, xylene, etc. Investigations in this art have shown that at any particular temperature and pressure, a mixture of hydrocarbons, or of hydrocarbons with free hydrogen or carbon, or both, tends to reach a 85 state of equilibrium at which definite quantities of the various materials will be present. A certain time, however, is required for the completion of the reaction, so that the state of equilibrium will not be attained if, within less than the time required for completion 90 of the reaction, fresh materials are added or portions of the materials withdrawn from the reaction zone. In consequence of the time-factor involved in the reaching of an 95 equilibrium, it is possible to vary the proportions of the resultant products of the "cracking" of higher hydrocarbons by varying the rate of feed, while the conditions of pressure and temperature are kept constant. 100

Applying the same reasoning to the decomposition of the higher hydrocarbons as employed in my carburizing process, it will be seen that by similar variation of the conditions, principally temperature and rate of 105 feed, a zone of reaction may be established and maintained substantially throughout the retort, wherein the resultant products are those which most highly favor the release of carbon in such a form or state as to penetrate and combine with the iron or ferric alloy. 110

I am aware that certain hydrocarbons have been employed in carburizing processes heretofore known, but in all such processes 115 where the hydrocarbon is fed continuously during the carburizing operation, a fixed and stabilized gas, generated outside of the retort has been employed. Ethane, methane, acetylene, ethylene, and other fixed hydro- 120 carbon gases, existing as such at ordinary temperatures, are known to be capable of effecting more or less carburization of iron when maintained in the presence thereof at suitable temperatures. Ethylene, in fact, 125

130

has been considered to be the fastest carburizing agent known, but has not been used extensively because the character of the case obtained therewith is not satisfactory for most uses. With ethylene, the case obtained is exceedingly abrupt, being hyper-eutectic with the carbon content ranging as high as 1.5 to 1.6% at the surface. For most commercial case-hardened work, it is desirable that the case at the surface should have a carbon-content not exceeding eutectic, and that there should be considerable penetration with a uniform and gradual reduction of the carbon-content from the surface inward. Carburization of this character is readily attained by my process, and is effected with remarkable rapidity. With specimens of soft steel, of .15% to .2% carbon-content, I have been able to carburize same to a depth of  $\frac{1}{8}$  inch or more by treatment for two hours at temperatures ranging around 1700° F., the case obtained having a carbon-content between .45% and eutectic, and not exceeding the latter at the surface. Moreover, the depth of penetration obtained is very nearly proportional to the length of the period of treatment, the penetration curve showing a gradual rise, and the rate not showing the marked slowing with increased penetration common to most carburizing processes. Carburizing by my process is not appreciably retarded by the presence of metals commonly alloyed with steel, such as chromium, vanadium, tungsten, manganese, or nickel. Nickel, for example, is shown to greatly retard carburization by ordinary methods, but with my process the carburization of nickel-steel may be effected at substantially the same rate as ordinary unalloyed or plain carbon steel.

As an example of the remarkable penetrative power of the carburizing substance or substances produced in carrying out my process, I may mention instances in which two plates were secured together by riveting, in order to prevent carburizing of their adjoining faces. After treatment of the plates thus secured together, examination thereof showed that carburization had been effected around the rivets for a considerable distance below the outer surface of the plates, the carburizing material apparently having penetrated the microscopic joint-space left after the upsetting and heading of the rivets. In the same examples, although the plates were held together by rivets and their edges cemented together, there was considerable penetration through the joint and into the back faces of the pairs of plates. From this it will be seen that agitation of the articles within the retort, or special arrangement thereof, other than to secure a slight separation of adjacent surfaces, is unnecessary to the securing of effective carburization.

65 I am at present unable to state definitely

what the material or materials are, which, being formed during the cracking and decomposition of the higher or complex hydrocarbons in carrying out my process, produce the carburizing effects attained by the process. It is certain, however, that the carburizing agent or agents are themselves hydrocarbons, since no other class of materials is present. It is fairly certain also that the effective agent or agents are not mere end-products of hydrocarbon decomposition, or the lower members of the hydrocarbon series, such as ethane, methane, ethylene, acetylene, etc., since these agents, by themselves or in any known combinations, cannot be made to effect the results attained by my process. It appears probable that the effective agent or agents are intermediate products, resulting from the progressive reduction of the higher and more complex hydrocarbons, and formed 75 transitorily in the reactions tending to produce a state of equilibrium at the temperatures employed in the process. It is noted that the end-products or equilibrium products resulting from continued treatment of 80 the higher hydrocarbons at the temperatures employed in the process, are free carbon, hydrogen, and the fixed gases which constitute the lowest members of the hydrocarbon series, particularly of the paraffins, olefins 85 and acetylenes. It seems probable that the effective carburizing agent or agents comprise a hydrocarbon vapor of such composition that under the conditions present in carrying out the process the material has an 90 extraordinary capability of penetrating the metal; that the said hydrocarbon, being unstable at the temperatures employed, undergoes a decomposition while in intimate or molecular contact with the metal, the decomposition being of such a nature as to release 95 carbon in a nascent or infra-molecular state, so that the released carbon unites with the metal and is retained thereby. The foregoing is offered merely as a working hypothesis 100 as to the nature of the reactions occurring, but is borne out by all experimental and other data now available.

An interesting indication of the nature of the reactions which occur in the retort during the carburizing process, is offered by the pyrometer readings when regulating the heat of the furnace to bring the same up or down to the temperature desired to be maintained, or when varying the rate of feeding 115 of oil to the retort. At temperature below about 1780° F., other conditions being uniform, increasing the rate of oil-feed causes a marked lowering of temperature in the retort, and decrease of rate of feed causes an 120 increase of temperature, so that apparently the reactions occurring are principally endothermic in character. It appears further that at temperatures approximating 1800° F. the reactions tend to become exothermic. 125 130

This is made evident by maintaining a uniform rate of oil-feed, and regulating the heating devices of the furnace so as to produce a gradual increase of temperature approaching the temperature last mentioned. At about 1800° the rate of increase will be noticeably accelerated, and upon reaching a temperature of 25 to 30 degrees higher said temperature will be maintained even though the furnace heating devices be shut down to a point which previously would serve only to maintain a temperature of the retort 100 or more degrees lower. In fact, after once bringing the retort-temperature up to the exothermic phase, it is sometimes difficult to secure a lowering of the temperature except by stopping the oil feed until the lowering is effected.

Now, having described my invention, what I claim and desire to secure by Letters Patent is:

1. The method of case-carburizing, consisting in heating the treated articles to and maintaining the same at a temperature above the critical temperature for hardening the material; and supplying with substantial continuity, so as to maintain about the heated articles a nearly uniform atmosphere thereof, a relatively complex hydrocarbon unstable at the maintained temperature of the articles.

2. The method of case-carburizing articles of steel, consisting in heating the same above the critical hardening temperature of the steel, in the presence of complex hydrocarbons which are unstable at the maintained temperature, whereby said hydrocarbons undergo constant decomposition of a character tending to free carbon therefrom, and supplying the hydrocarbons at a controlled rate, whereby to maintain a substantially constant reaction zone about the articles.

3. The method of case-carburizing articles of iron and steel, consisting in heating and maintaining the same at temperatures ranging upward from the critical temperature of the material, in a constantly replenished atmosphere consisting principally of intermediate decomposition products of complex higher hydrocarbons.

4. The method of case-carburizing articles of iron, steel and alloys thereof, consisting in heating the articles in an atmosphere consisting principally of petroleum decomposi-

tion products, and discharging said decomposition products from the reaction zone containing the treated articles, at a rate such as to substantially exclude from said zone the decomposition end-products other than carbon.

5. The method of carburizing articles of iron, steel and alloys thereof; consisting in decomposing normally liquid hydrocarbons by abruptly subjecting the same to temperatures high enough to release carbon therefrom, placing the articles to be carburized in the zone of said decomposition, and controlling the rate of feed of the hydrocarbons to and of escape of the decomposition products from said zone so as to maintain a substantially constant reaction therein.

6. The method of carburizing articles of iron, steel and alloys thereof, consisting in passing normally liquid petroleum products abruptly into a zone of high temperatures such as to decompose and release carbon therefrom, placing the articles to be carburized in the zone of reaction in which carbon is being released, and maintaining a substantially constant rate of feed and escape of the materials to and from said zone of reaction.

7. The method of carburizing articles of iron, steel and alloys thereof, consisting in heating the articles to carburizing temperatures in a current of relatively complex hydrocarbons unstable at the maintained temperature, and so controlling the rate of flow of said current as to maintain about the articles a reaction zone in which the decomposition products are intermediate the initial hydrocarbons and the end-products of decomposition thereof at the maintained temperatures and pressures.

8. The method of carburizing articles of iron, steel and alloys thereof, consisting in heating the articles to carburizing temperatures in a current of normally liquid petroleum products which are unstable at the maintained temperature, and so controlling the rate of flow of said current as to maintain about the articles a substantially constant reaction zone containing decomposition products intermediate the initial and end-products of decomposition of the material at the maintained temperatures and pressures.

A. J. P. BERTSCHY.